

May 3, 1932.

H. M. WILLIAMS ET AL

1,856,679

APPARATUS FOR COMMINUTING METALS

Filed July 22, 1925 2 Sheets-Sheet 1



Inventors

H. M. Williams  
and V. W. Bihlman,  
By Spencer, Sewall & Hardman,  
their Attorneys.

May 3, 1932.

H. M. WILLIAMS ET AL

1,856,679

## APPARATUS FOR COMMINUTING METALS

Filed July 22, 1925 2 Sheets-Sheet 2



### Inventors

R. M. Williams  
and V. W. Buhlman  
by Spencer, Gerald & Hardman  
their Attorneys

## UNITED STATES PATENT OFFICE

ARRY M. WILLIAMS AND VICTOR W. BIHLMAN, OF DAYTON, OHIO, ASSIGNORS TO  
GENERAL MOTORS RESEARCH CORPORATION, A CORPORATION OF DELAWARE

## APPARATUS FOR COMMINUTING METALS

Application filed July 22, 1925. Serial No. 45,284.

This invention relates to the comminuting of metals of relatively high melting point, by atomizing them while in a molten condition, by a stream of aeriform fluid under pressure.

- 5 It has hitherto been proposed to atomize metals of relatively low melting point by melting them, letting the molten metal flow through a nozzle and forcing a stream of air or steam into contact with the stream of 10 molten metal. This process has been commercially practiced with lead, tin and other metals of relatively low melting point. So far as I am aware, metals of high melting point, such as copper, nickel and the like, have 15 never been commercially produced by this method.

It is an object of this invention to produce metallic powders of copper, or other high-melting-point metals, by atomization.

- 20 The invention consists in the method of atomizing high-melting-point metals, and in an apparatus for carrying out this method, as more fully described hereinafter, illustrated in the accompanying drawings, and 25 defined in the appended claims.

In the drawings, in which like reference characters indicate like parts throughout the several views:

30 Fig. 1 is an elevation, partly in section, of an apparatus adapted to practice the process of this invention;

35 Fig. 2 is a section through a fragment of a furnace, crucible and atomizing nozzle, forming part of the invention;

Fig. 3 is a section of a fragment taken on the line 3—3 of Fig. 2, looking upward toward the bottom of the furnace and crucible; and

40 Fig. 4 is a view similar to Fig. 3, showing a modification in the relation of the inlet pipes to the atomizing nozzles.

In Fig. 1, 10 indicates a furnace which may be of the combustion type, fed by combustible gas through a pipe 11. A removable cover 45 12 normally closes the upper end of said furnace, this cover may have a hole in it (not shown) for receiving a funnel by means of which to guide molten metal into a crucible disposed in the interior thereof, as will be 50 explained presently. The furnace 10 has an

opening in its bottom communicating with an expansion space in a large pipe 13 beneath it. Pipe 13 is closed at its upper end excepting that it has an opening registering with the opening in the furnace. The pipe 13, as shown in Fig. 1, curves to one side at 14, and enters the lower portion of a large collection chamber 15 having an inclined bottom 16, a top 17 which is open to the atmosphere, preferably through a fine-meshed fabric to prevent metallic dust leaving the chamber 15 through the top. At the lower end of the inclined part 16, there is a door 18, through which copper or other metallic powder, produced by the atomizing process to be described, may be removed.

The furnace 10 may be built up of fire brick 19, or other refractory material, within a shell of metal 20, and may be supplied with combustible gas through pipe 11 at any suitable point, preferably just above the ledge 19a, which may be formed of fire clay, or the like. The ledge of fire clay 19a is of annular form, the opening in it being lined with a collar 21 having an internal flange 22. The opening within the flange 22 of said collar 21 is occupied by a bottom member 23, having a flange 24, resting upon the flange 22. Said bottom member 23 has a central hole 25 and one or more smaller holes 26, arranged around it. The collar 21 and the bottom member 23 may be made of cast iron, or preferably of some suitable high-heat-resisting material, such as nichrome.

Resting within the furnace 10 is a crucible 27 made of any of the usual materials adapted for the purpose, such as graphite. In the form shown in Fig. 2, the crucible 27 has an extension 28 of the same material, which is screw-threaded into the bottom of the crucible, as at 29, or may also be integral with it. The extension 28 tapers downward and the lower end rests upon the bottom plate 23, said extension having an opening in its lower end registering with the opening 25. Into the lower end of extension 28, there is secured, as by screw threads 30, a graphite nozzle 31 which has a tapering lower end protruding some distance below the extension 28, and an upper end extending some distance up into

55

60

65

70

75

80

85

90

95

100

said extension. The lower tapering end of the nozzle is pierced to receive a tube 32 made up of any suitable material, as quartz or lavite, said tube being suitably secured in place. Above the quartz tube the graphite nozzle is counterbored as at 33, the upper end of the counterbore being closed by a cap 34, also of graphite. The walls of the graphite nozzle 31 are perforated as at 35, to form 10 passages for the entrance of molten metal from the crucible into the nozzle. Because of the presence of passages 35 the nozzle acts as a strainer to prevent the entrance into the nozzle of dross, slag, or other coarse material, which might act to clog the quartz tube 32.

The lower end of nozzle 31 protrudes some little distance below the lower side of the furnace, through the opening 25 in the bottom 20 plate 23. This end of the nozzle is encased by a shell 36 of heat-resistant metal, to mechanically strengthen the graphite and prevent burning. Surrounding the protruding end of the nozzle, is an annular nozzle for 25 receiving aeriform fluid under pressure, such as air, and discharging it in a converging stream, annular in cross-section, around the exit of the quartz tube 32. This annular nozzle will be termed, for convenience, an "air 30 nozzle". The main part of the air nozzle is indicated in Fig. 2 by the numeral 37. The inner part of it comprises a shell 38 which conforms, interiorly, substantially to the shell 36, but is spaced slightly therefrom in order 35 that there may be no binding because of warping or expansion due to heat. The said members 36, 37 and 38, should be of high-heat-resisting metal, and we have found that an alloy known commercially as "Resistal", 40 is well-suited for the purpose. Tapped into the member 37 of the annular air nozzle, are pipes 39 leading from a source (not shown) of air, or other suitable gaseous material, under pressure. The air nozzle may be secured in place by any suitable means, iron bolts 40, as shown in Fig. 2, answer the purpose 45 very well; although they may have to be replaced occasionally, owing to the destructive effect of heat to which they are subjected.

Surrounding the air nozzle and secured to the bottom plate 23, by said bolts 40 and nuts 41, is a casing 42 made of sheet metal of suitable high-heat-resisting material, which 55 may be Resistal, or a metal known commercially as "Ascoloy". Pipes 39 penetrate the wall of the casing 42 and fit snugly therein. When the casing 42 is in place, it is in communication with the interior of the furnace 60 10, by means of openings 26, so that it will be seen, when combustion is taking place within the furnace 10, products of combustion will enter the chamber within the casing 42, circulate around the nozzles, and that 65 some of the products of combustion may pass

out through a central opening 43 formed in the bottom of the casing 42, in concentric registration with the quartz tube 32 and the annular atomizing orifice, indicated by the numeral 44.

Instead of having the pipes for conducting aeriform fluid under pressure with the air nozzle arranged radially, as indicated in Figs. 2 and 3, the air-conducting pipes may enter the annular space between the elements 37 and 38 of the air nozzle in a tangential direction so as to cause the aeriform fluid to issue from the annular orifice 44 in a whirling state. In Fig. 4 the air-conducting pipes 39a are shown disposed tangentially 75 to effect increased agitation of the stream of molten metal where the air acts upon it.

In the practice of this method, copper or other relatively high-melting-point metal is brought to a state of fusion in any suitable 80 way. The furnace 10 is preheated to a high degree of heat by starting combustion well in advance of the time of filling the crucible 27 with the molten metal, so that the crucible is heated to a high temperature and 85 products of combustion circulating around the nozzle portions exteriorly of the furnace, said nozzle portions are also preheated to a relatively high temperature, say, from 1600 to 2000 degrees Fahrenheit, more or less. 90 When crucible and nozzles have been brought to the required temperature, the molten metal heated in another furnace is conducted to the heated crucible 27. From said heated crucible, the molten metal flows through the 95 small passages 35 into the interior of the nozzle 31 and thence passes, free from dross or slag, into and through the quartz tube 32. While the molten metal is issuing from the 100 quartz tube 32, the atomizing fluid is forced by pipes 39 into the annular nozzle and out through the annular opening 44, beyond which the end of the quartz tube 32 protrudes 105 slightly. The atomizing fluid takes an inverse conoidal form, surrounding the stream of molten metal, which falls substantially into the apex of the cone. This stream has an entraining action tending to withdraw 110 molten metal from the crucible. The impact of the atomizing fluid and the sudden expansion of it, as it loses its force in the large 115 expansion space afforded by the pipe 13, breaks up the stream of metal into fine particles, which fall down the pipe and progress toward the door 18. The powder of copper 120 and other metals thus produced, may be swept from the walls of the pipe 13, and the chamber 15, and collected adjacent the door 18, from which it may be removed.

It is found in the treatment of copper, 125 that a large proportion of the powder, approximately 75%, is of a size to pass through a 200-mesh sieve, and that the powder of this fineness is pure copper, substantially free from oxide, while the coarser particles are 130

found to be oxidized, more or less, and not usable where pure copper powders are needed, as in the manufacture of bushings, brushes, and the like.

5 While the form of embodiment of the invention as herein disclosed, constitutes a preferred form, it is to be understood that other forms might be adopted, all coming within the scope of the claims which follow.

10 What is claimed is as follows:

1. Apparatus for producing metallic powders of relatively high-melting-point metals comprising, in combination, a furnace, a crucible in which the metal is melted, a nozzle 15 connected with the crucible and extending outside the furnace, means for directing the gaseous products of combustion from said furnace around the discharge end of the nozzle to maintain the nozzle at a relatively high 20 temperature and means for subjecting the metal issuing from the nozzle to a whirling stream of aeriform fluid under pressure and causing the products of combustion to flow around the part of said nozzle outside the 25 furnace.

2. Apparatus for producing metallic powders of relatively high-melting-point metals comprising, in combination, a furnace, a crucible in which the metal is melted, a nozzle 30 connected with the crucible and extending outside the furnace, means for directing the gaseous products of combustion from said furnace around the discharge end of the nozzle to maintain the nozzle at a relatively high 35 temperature and means for subjecting the metal issuing from the nozzle to a hollow stream of aeriform fluid under pressure surrounding said nozzle and causing the products of combustion to flow around the part of 40 said nozzle outside the furnace.

3. The combination of a furnace having an opening, a crucible disposed within the furnace, a nozzle connected to the crucible extending through said opening, said nozzle 45 having perforations adapted to function as a strainer of the metal entering the nozzle, and means for atomizing the metal issuing from the nozzle by a stream of aeriform fluid under pressure.

50 4. The combination of a furnace having a bottom plate provided with an orifice, a crucible disposed within said furnace, a nozzle connected to the crucible and extending through the orifice in said plate, means for 55 atomizing the metal issuing from said nozzle, said means and nozzle being encased within a casing which communicates with the interior of the furnace and has an opening with which the atomizing orifices register.

60 5. In means for atomizing metals, a crucible having a graphite nozzle provided with a quartz exit tube.

65 6. In means for atomizing metals, a crucible having a graphite nozzle projecting some distance into the crucible and having

perforations in its side adapted to strain the metal entering it.

7. Apparatus for producing metallic powders of relatively high melting point metals comprising a nozzle, means for preheating the nozzle to a relatively high temperature, means for conducting metal in a molten state to the nozzle, means for filtering the metal before its admission to the nozzle, and means for directing a stream of aeriform fluid under pressure against the metal issuing from the nozzle whereby it is atomized.

In testimony whereof we hereto affix our signatures.

HARRY M. WILLIAMS. 80  
VICTOR W. BIHLMAN.

85

90

95

100

105

110

115

120

125

130